

## UNITED STATES PATENT OFFICE

2,429,644

## ART OF ESTERIFICATION

William Beach Pratt, deceased, late of Boston, Mass., by Annette Harris Pratt, administratrix, Boston, Mass., assignor, by mesne assignments, to Joseph G. Denny, Jr.

No Drawing. Application August 8, 1940,  
Serial No. 351,912

8 Claims. (Cl. 8-121)

1

Broadly speaking, this invention relates to esterification with organic acids and anhydrides, or mixtures of the same, particularly to the esterification of cellulose, starch, dextrins and other carbohydrate bodies preferably in their natural or normal state, as individual fibers, granules, fiber aggregates as woven goods, cloth, textiles or twisted or untwisted rovings and yarn, composed wholly or partially of cellulose.

This invention involves novel procedure and compounds used in the formation of valuable products, and especially applicable wherein the original appearance of the fiber or granule may or may not be materially modified in appearance by transformation into the corresponding ester form, and whereby the toughness, flexibility and elasticity of the esterified carbohydrate in nearly every instance is at least equal to the original body from which the ester has been prepared, especially when the natural carbohydrate is a fiber or filament prior to esterification.

In general, the practice of this invention involves treatment of a single or mixed carbohydrate, as normal, natural cellulose, as distinguished from hydrocellulose, hydrated cellulose, oxycellulose, degraded or otherwise modified normal cellulose, or there may be used a mixture of celluloses with other fibrous bodies, said carbohydrate being in the substantially anhydrous condition when catalysts, diluents and/or reactants are contacted therewith, and initially treat the same with a body or bodies having catalytic functions, dissolved or suspended in a neutral volatile liquid, which liquid may be an ester or susceptible to esterification in the carbohydrate esterifying bath, to an ester of the same acid radical as the carbohydrate esterified, yet in the esterified condition is usually substantially a non-solvent, or at best a poor solvent of the carbohydrate ester formed.

Where cellulose in some form is the carbohydrate to be esterified, it is preferred to employ natural or normal cellulose in the fibrous state, as linters, fly, rovings, staple, woven, sheeted or pressed form, as yarn, cloth or textiles, and from which substantially all atmospheric moisture has been removed at the time the cellulose is initially treated.

If woven or textile fibers are to be esterified and with little or no observable change in form, structure or appearance during esterification, there may be employed a textile wholly of natural cellulose fibers, or a mixture including mercerized or other treated or modified cellulosic fibers, or a

2

mixture of cellulosic natural fibers with other fibers containing nitrogen, as wool or silk.

As catalyst there is employed a body in the liquid or solid state, or a plurality of suitable dissimilar bodies, which are partially or totally soluble in or miscible with an aliphatic hydroxide or hydroxides, or mixture of similar or dissimilar aliphatic hydroxides with aliphatic oxides, and which are substantially anhydrous when used as catalyst solvent or diluent, which comprise in the hydroxide form less than five atoms of carbon, or in the oxide form less than ten carbon atoms, and which are soluble in or partially miscible with water, and are also capable of esterification in the same bath in which the carbohydrate is being esterified, but which aliphatic ester when formed is a non-solvent or at best a weak solvent of the esterified carbohydrate, thus permitting said carbohydrate to be esterified under normal pressure and tension without appreciable change in physical form or appearance.

Where an aliphatic hydroxide of more than five carbon atoms or the corresponding aliphatic oxide of more than ten carbon atoms are employed alone or admixed with an aliphatic hydroxide, or oxide of lesser carbon content, in general, less satisfactory results have been obtained.

As aliphatic hydroxide, oxide or ester, there may be used methyl alcohol or ethyl alcohol as examples, either alone or admixed together in various proportions, or with a proportion of the corresponding or other oxide, as diethyl oxide,  $(C_2H_5)_2O$ , or an alkyl ester of an aliphatic monocarboxylic acid as methyl or ethyl acetates.

Or, there may be used a higher alcohol mixed with a lower one as iso-propyl and methyl alcohol, but it is preferable that the liquid be substantially anhydrous when catalyst is dissolved therein or mixed therewith and the mixture contacted with the carbohydrate.

As catalyst there may be employed any suitable halogen (except fluorine) oxyacid or anhydride or the same including perchloric acid as set out in an application of W. B. Pratt, Serial No. 289,712, filed Aug. 11, 1939, or mixtures of halogen oxyacids of same or dissimilar oxygen content, but preferably of relatively high oxygen content, which is or are miscible with or soluble in the above mentioned aliphatic alcohols, esters or mixtures thereof.

As a specific example of "relatively high oxygen content," satisfactory results may be obtained by the use of bromic or perbromic acid, or their anhydrides bromine pentoxide (bromic anhydride) or bromine heptoxide (perbromic anhydride) as

distinguished from the lower oxyacids, bromous or hypobromous, or their respective anhydrides, and less satisfactory effects result from the use of corresponding oxyacids, containing not less than three oxygen atoms of the halogens bromine and iodine or their corresponding anhydrides, or of chloric acid, alone or in admixture.

According to this invention, best results are obtainable when operating with the carbohydrates in their different variations and forms, by impregnating the carbohydrate with the halogen oxyacid, the selection of most suitable halogen oxyacid catalyst or mixture thereof in esterifying a particular carbohydrate body, depending in a measure upon the nature, source, form and other characteristics in the carbohydrate initially used, and the form and physical properties desired in the finished esterified product.

A catalyst of or containing a major proportion of bromic acid, or a mixture of bromic and iodic acids is desirable.

One preferred method of practice of this invention taking the carbohydrate group as a whole involves impregnating a substantially anhydrous aliphatic monohydric alcohol containing a halogen oxyacid of relatively high oxygen content, as bromic acid in the hydrate form, thus forming a relatively fixed "constant boiling acid" soluble in the monohydric alcohol, and which is convertible by dehydration into a more or less volatile oxide as bromine pentoxide which appears in general to be more effective as an esterification catalyst than the original halogen hydroxy acid.

The mechanics of this invention appear to be that the impregnation of the carbohydrate with alkyl hydroxide or oxide devoid of water repellents improves the uniformity of the wetting of the carbohydrate by water of reaction subsequently formed in situ therein and places it on the same phase of reaction as a suitable substantially anhydrous dehydrating and esterifying reagent, such as an aliphatic acid anhydride, as acetic anhydride.

The anhydride reacts with the hydrous catalyst to apparently form a volatile and more effective catalyst such perhaps as bromine pentoxide; reacts with the alcohol to form water and a diluent of the anhydride used to esterify the alcohol to the corresponding ester; and reacts rapidly and uniformly upon the activated carbohydrate to form an ester, as acetylcellulose.

The catalyst thus formed in situ, or in the nascent state as it were, in the carbohydrate is unstable in the presence of an oxidant or oxidizable material such as cellulose, and is stabilized during esterification of the carbohydrate and thereafter removed from the formed ester as by an evaporative step, thereby preventing degeneration and hence requiring little or no washing.

The stabilization of the relatively unstable catalyst is preferably effected by maintaining air or other source of oxygen in contact therewith, for a portion of the time, or throughout the esterification phase.

The principal of this invention is intimately connected with the relative amounts and distribution of water, and minimum amounts of water in each of the entering components, and in each phase of the treatment of carbohydrate initially until the close of the esterification step. There should be some moisture present to initiate esterification, after which sufficient water is obtained by virtue of hydroxyl in the alcohol and the hydroxyl in the carbohydrate incident to aceta-

acids or anhydrides or both. The moisture originally present in the carbohydrate just prior to initiation of esterification and which preferably should be less than one percent as determined by dehydrating at 105°-110° C., coupled with the relatively small amount of water in the catalytic body as initially introduced into contact with the cellulose, may supply the water to initiate esterification of the alcohol under the conditions prevailing, and this amount of water is usually deemed sufficient, due to the increased receptivity, and increased uniformity of receptivity of the carbohydrate for esterification reaction, by virtue of the commingling of catalyst and carbohydrate under the conditions herein set forth.

Esterification is greatly facilitated, accelerated and rendered more uniform by virtue of the presence of the halogen oxyacid anhydride as bromine pentoxide, as inducing and continuing esterification under the conditions prevailing. Such bromine pentoxide has no apparent injurious effects, due primarily to its proneness to evaporate and completely volatilize from the treated carbohydrate at the close of the esterification. The presence therein of the neutral, volatile, cellulose ester diluent in ester form, also modifies and lessens danger of untoward effect upon carbohydrate at the initial point of esterification, and during the esterifying cycle.

The bromine pentoxide is preferably formed in situ and is preferably effected by the reaction of an esterifying anhydride on a bromic acid hydrate containing a proportion of moisture, say of 60% to 80% absolute HBrO<sub>3</sub>, and about two molecules of water, and which is capable of holding 1-1.5 additional molecules of water.

Such bromic acid hydrate appears to be stable to light and mechanical shock; is soluble in or miscible with the aliphatic alcohols or esters mentioned herein, and has a relatively low boiling point. It therefore will not vaporize from the cellulose or fabric to any considerable extent under the conditions to which the fabric is treated prior to esterification.

For purposes of description, this invention may be said to involve two steps, both carried out with substantially anhydrous materials as expressed in percentage of the combined reactants, and as follows:

(1) Treatment of carbohydrate prior to esterification with catalyst associated with alkyl hydroxide, with or without alkyl acetate.

(2) Contacting treated carbohydrate with ester-forming components.

(1) *Preliminary treatment of carbohydrate.*—For purposes of illustration only, one exemplification of this process will be described as of treatment of normal cellulose in the fibrous form and in the textile condition, as muslin, linen, duck, drill, canvas or other form, weight, weave or weft or suitably purified cellulose fiber.

The catalyst selected is first dissolved or suspended in the proportion desired in the alkyl hydroxide or ester or mixture thereof, or mixture of alkyl hydroxides, with or without the addition of an alkyl ester thereto, all in the substantially anhydrous condition.

Synthetic methanol alone or with a proportion of ethyl ether, or "absolute" ethanol, in general has been found preferable, especially when a fibrous carbohydrate carboxylate is to be the finished ester.

If upon contact of catalyst with alkyl hydroxide, too much heat is evolved as the result, the mixture may be cooled before use, or the alkyl

hydroxide may be cooled before admixture of catalyst therewith. Catalyst in solution or suspension or both, is then contacted with the carbohydrate, either at room or elevated temperatures, and allowed to remain in contact therewith for a period of time, from a few minutes up to several hours, depending in a measure upon the amount and nature of the catalyst employed, and the kind and relative purity of carbohydrate used.

The composition may be agitated during the preliminary carbohydrate treatment step if desired, and it has been found advisable to limit contact with normal air on account of moisture absorption to an unknown and variable degree.

No esterifying acid or anhydride or water repellent agent is used in this preliminary carbohydrate treatment step.

In another variation of the process for esterifying cloth according to this invention, an ordinary padding machine may be used to immerse the dehydrated carbohydrate in the aliphatic alcohol in which there has been thoroughly mixed the halogen acid as bromic acid. There is no apparent reaction between the bromic acid where methanol is used, or on cellulose in this treatment, even at the boiling point of methanol.

The methanol uniformly dispersed the catalyst throughout and in the interior of the cellulose fibers, and removes, unifies, disperses or equalizes the distribution of the remaining variable amounts of water moisture from the cellulose, but does not seem to remove the water of hydration from the halogen oxyacid used, at least to any observable degree.

Speaking of normal cotton cellulose, saturation point of the cellulose fibers is about 62% of their weight of methanol and about 1.3-1.6% of their weight of bromic acid, which is selectively not absorbed from the methanol. Such a high methanol content is usually not necessary, and generally is undesirable for esterification, since the amount of methanol carrying catalyst left in the fibers should normally be only sufficient to form by reaction with anhydride sufficient water for initiation of cellulose esterification.

Consequently the saturated cellulose, after having passed through squeeze rolls, is subjected to an evaporative step until the methanol content is reduced by evaporation to between 10% and 30%, preferably to about 20% to 25%, based on the dry weight of the cellulose.

Or, in a modification of this step, the amount of methanol used may be just sufficient to produce the desired amount of methyl ester in the acetation step, and the difference in liquid associated with catalyst in the carbohydrate pre-treatment step may be a monohydric aliphatic ester, such as methyl acetate. In such case, the step of removal of methyl hydroxide to the degree desired for hydroxyl elimination in the subsequent acetation step is unnecessary.

The bromic acid content appears unaffected by the drying step and remains about 1.1-1.7% of the weight of the cellulose.

Contact of catalyst in neutral, anhydrous liquid with dry carbohydrate, causes uniform and complete penetration throughout the filamentous mass, including filling the filamentous lumen of the individual cotton fiber with liquid containing catalyst evenly and intimately dissolved therein and distributed therethrough. The cellulose is thereby rendered more reactive and more uniformly receptive to subsequent esterification, and the esterification is carried out in a more uniform manner and is less time-consuming, thereby pro-

ducing a product of relatively high stability and yield.

The catalyst solvent containing hydroxyl in conjunction with the relatively small amount of moisture still normally retained in the cellulose if such moisture there now be, admits of initiation of esterification, and in a manner without observable local rise of temperature, due to this uniform prior dissemination and dispersion to an almost intermolecular degree and actual interpenetration of catalyst into cellulose substance.

That is, at the moment of commencement of esterification when initiated under the conditions as described herein as prevailing, each cellulosic entity is permeated and saturated in a uniform manner with the same proportions or amount of catalytically-acting body.

This obviates the possibility of serious localized reactions and an irregular rate of esterification with corresponding formation of a series of different carbohydrate organic acid esters, as cellulose acetates, as determined by varying amount of acetyl associated with the cellulose, such localized reactions being always accompanied by rise in temperature and disintegration and degradation of the cellulose.

It has been discovered as a generality, that localized and irregular reactions during esterification are due primarily to irregular distribution of water occluded in, or physically or chemically combined with, the cellulose or the esterifying bath components.

While the presence of water is essential to esterification, especially in its first phases, it has been demonstrated that its action can effectively be controlled primarily if not only by the formation thereof by reaction in situ, and that all of the components present and involved in the esterification of the cellulose, should be initially so anhydrous that their determinable aggregate water contact is initially insufficient to initiate esterification in the treated cellulose or to set up observable local reaction.

The preferred practice of this invention therefore, requires exclusion of water to the utmost degree possible from the esterifying substances, and especially the uniform displacement, diffusion and dissemination of minute quantities of extraneous water that may remain. And the development by reaction, of water in situ in the molecular structure of the cellulose is sufficient, once esterification is initiated under these conditions to continue cellulose esterification uniformly to a product of substantially maximum degree of combination of cellulose with acetyl. Such water of reaction in contradistinction to small amounts of water originally present in the cellulose or reactants, is generated by the esterification of the water-soluble aliphatic alcohol or alcohol and ether, which more readily esterifies than does the cellulose, such esterification producing an ester which is a diluent but a non-solvent of the acetated cellulose upon formation.

The preliminary esterification of the alcohol appears to take place, at least in its first phases, immediately prior to, or concurrently with the esterification of the cellulose and in intimate contact with the structure thereof. The much smaller molecular weight of the aliphatic alcohol in comparison to the relatively huge cellulosic aggregate, causes initiation of esterification first in the alcohol and releases water to initiate esterification of the carbohydrate and to assist in the continuation of that esterification.

The removal of the practically all free or originally uncombined water, including physically attached or chemically combined water (so-called water or constitution) from the carbohydrate, as cellulose, and the complete and uniform impregnation of its molecular structure with anhydrous aliphatic hydroxide, places the cellulose in the same phase or zone of reaction as the water-free esterifying bath. Even if the esterifying bath originally contained small amounts of water, the probability is that it would first be combined with the acid anhydride to form the corresponding acid.

By thus eliminating any interfacial tension between the constituents of the esterifying bath and the products to be esterified, the latter are completely, uniformly and substantially instantaneously penetrated and impregnated by the former, so that the esterifying reaction proceeds uniformly under these conditions throughout the molecular cellulosic structure.

By thus observing the prior outlined conditions, this permits of substantially instantaneous subsequent esterification perfectly uniform throughout, and hence with no observable appreciable degradation of cellulose in passing from the normal into the ester form, thereby assuring that the cellulose ester so formed shall retain its original desirable physical characteristics as tensile strength not only substantially unimpaired, but appreciably augmented, sometimes up to 50% increase and more.

This includes toughness, elasticity, flexibility, resiliency, tensile strength and uniformity of gelatinization, colloidation and solution in a wide variety of solvents, solvent combinations, diluents, flexilizers, plasticizers and supple-inducing bodies.

Such acetylated celluloses in the fabric form possess the desirable qualities to a much greater degree than do yarns and fabrics made from or containing hydrolyzed, degenerated or oxidized cellulose, either before or after esterification thereof.

The esterification of celluloses according to this invention, especially after the cellulose filaments have been spun into yarn or woven into fabric, results in an increase in diameter of the individual filament, an increase in number of turns or twists per inch in the yarn, and the relative transparency, translucency, opacity, luster and other properties of such acetylated yarns or fabrics made therefrom, may be largely modified and controlled by the degree of tension applied thereto in one or more directions during the esterification and subsequent treatments and usually until the finished fabric has assumed the air-dry condition.

The weight of the carbohydrate is also increased incident to acetylation by this invention, up to 50%, and even more.

After contact of catalyst and cellulose in the presence of an aliphatic hydroxide or oxide or mixture thereof, or a body possessing alcoholic functions, for the length of time required to assure complete and uniform association and permeation of catalyst of the nature as herein disclosed with and into the cellulose, either at rest or with agitation, excess of liquid and catalyst is removed in any convenient manner, as by pressure, centrifugalization or evaporation, and until the original cellulose shows a gain in weight of not to exceed about 30%, when it is immediately, or after maturing, contacted with esterifying components.

(2) *Esterification of preliminary treated cellu-*

*lose.*—The esterifying bath comprises the anhydride of the organic acid sought to be introduced into the carbohydrate aggregate, of substantially anhydrous concentration, and preferably with little or no corresponding acid being used.

Where it is desired to obtain the carbohydrate ester in the original granular (as with starch) or filamentous (as with the cellulose) form, the esterifying bath should contain a proportion of inert diluent or carbohydrate ester non-solvent, which non-solvent for purposes of economy and subsequent recovery may be the same ester as that formed by introduction of the alcohol in the prior pretreatment step, after that alcohol or ether is subjected to esterification.

If acetylation of cellulose is desired and ethanol has been used as the vehicle to contact cellulose and catalyst, then the esterifying bath is preferably composed of or contains the aliphatic acid anhydride as acetic anhydride, with ethyl acetate as non-solvent or diluent for the acetylated cellulose formed.

If the ethanol above has been replaced by a mixture of ethanol and ethyl acetate or methanol and methyl acetate, then the esterifying bath diluent may be either methyl acetate, ethyl acetate or a mixture of the same in the desired proportions.

If the process is to be a more or less continuous one as where rolls of textiles are to be esterified, then the textile is preferably placed under tension, either or both longitudinal or lateral, the degree of tension employed in either or both directions being determined by the properties desired in the esterified textile. Cotton or linen textile, or a mixture of mercerized and non-mercerized cotton fibers undergo considerable contraction upon being esterified in accordance with this invention. The stresses on the textiles are preferably gradually decreased during the early stages of esterification and gradually increased during the later stages of esterification by varying the tension applied to the textile.

Where relatively considerable tension is employed, it has been found that certain physical properties as luster are profoundly modified, esterification proceeding more speedily and uniformly when considerable tension is applied to the fabric, perhaps due to more readily penetration in the textile of esterifying agent in the stretched condition.

Esterification of carbohydrates, particularly cellulose and readily noticeable in the fabric form, causes a distinct tautening and contraction, and variation in tension or degree of tension imposed during the esterifying step, produces corresponding results in appearance of the finished product, especially in augmentation of the sheen, feel and facility of penetration of dyestuff and other treating materials normally applied to cellulose goods.

After contact of esterifying liquid with cellulose for the period required to produce the degree of esterification desired, and preferably in the presence of a source of oxygen, fabric is removed from the zone of further esterification, reactants removed therefrom as by washing or a solvent recovery step, and the fabric freed from excess moisture, as by passing through a dryer, still under tension, or the tension may be partially or wholly removed therefrom.

In lieu of acetic anhydride, other esterifying anhydrides or anhydrous fatty acids may be used, as formic acid, propionic anhydride, propionic

acid, or mixtures thereof, where a mixed carbohydrate ester is to be produced.

This method permits the use of amounts of esterifying acids or anhydrides in such slight excess of the amounts theoretically required for reaction with the alcohol or alcohol and ether and with the cellulose, that uniform mono-, di- and tri-esters of cellulose, broadly speaking, may be directly produced by properly proportioning the amount of the esterifying anhydride or acid or both, to the alcohol and cellulose, and control of the temperature and other constants during esterification, thereby avoiding or minimizing necessity for hydrolyzing or saponifying the primary ester to secondary ester, unless so desired.

Factors governing the percentages of acetic anhydride usually necessary for the formation of a desired primary or secondary cellulose acetate, the reactions involved, and controls desirable in commercial practice are illustrated by the following table applicable to the introduction into acetic anhydride of 100 pounds of cellulose containing 30% methanol and catalyst as hereinbefore set forth:

|                                                                          |      |
|--------------------------------------------------------------------------|------|
| Pounds of water formed                                                   | 8.46 |
| Pounds of methyl acetate formed                                          | 69.3 |
| Pounds of 100% acetic anhydride hydrolyzed by the water formed           | 48.0 |
| Pounds of acetic acid formed from the hydrolysis of the acetic anhydride | 56.4 |

To form cellulose triacetate (based on a C<sub>6</sub> cellulose molecule) under such conditions, there theoretically should be initially present not less than 293 pounds of acetic anhydride; or to form cellulose diacetate there should be initially present not less than 227.3 pounds of acetic anhydride; or to form cellulose monoacetate there should be initially present not less than 161.6 pounds of acetic anhydride.

In commercial practice it is advantageous to use approximately 10% or more in excess of the amounts of acetic anhydride theoretically indicated, but this amount is susceptible to considerable variation depending upon the condition and nature of the carbohydrate at the time of esterification, the temperature of esterification, and the particular halogen hydroxy acid used as catalyst.

The uniform saturation of fibers with such small amounts of anhydride is difficult, hence it is generally desirable to add to the anhydride a sufficient quantity of diluent to initiate, facilitate, control and unify reaction. When the cellulose is simply passed through the esterification bath and the reaction completed during the movement of the cellulose through the air, much less diluent is required than when the cellulose is completely esterified in the bath.

When it is desired to form a cellulose ester in solution rather than maintain the structural identity of the fibers, the diluent may comprise or contain a solvent for the particular cellulose acetate being formed, as for instance, acetic acid may be used as diluent when cellulose acetate in solution in the esterizing bath is desired, or a polyhydric alcohol may be used as the hydroxide for bringing the catalyst in contact with the cellulose. As example, if a dihydric alcohol as glycol, or a trihydric alcohol as glycerol be employed, the acetylated glycol or acetylated glycerol formed in the acetylating bath has solvent effect upon the carbohydrate ester formed.

*Example 1.—Acetation of linters.* As a quantitative illustration of one method of carrying

this invention into effect and as applied to cellulose as the carbohydrate in the non-woven condition, the cellulose as linters properly purified, is rendered "bone dry" or slightly drier by removal of moisture therefrom and until the moisture content is preferably below 1%, allowed to cool, and kept in a dry atmosphere.

To 100 parts of such cellulose is added 1.5-2.5% of bromic acid of 60% to 80% strength, dissolved in or admixed with anhydrous methyl alcohol, at least equal in weight to the weight of the cellulose to be treated.

The addition of dissolved catalyst is made to cellulose at normal or elevated temperature, and the mass stirred or otherwise agitated for several hours. Contact of cellulose and catalyst is maintained preferably in a closed container to prevent or minimize absorption of atmospheric moisture, unless the atmosphere has been dehumidified.

The cellulose and catalyst may be allowed to remain at rest for a further period if desired, to ensure maximum reactivity to be imparted to the cellulose.

At the close of the "steeping," "maturing," "activation" or intermingling step, the cellulose is then reduced in alcohol content to 20% to 30% increase in weight of the cellulose, preferably about 25% by weight, by a pressure, evaporative or centrifugal operation, and then immersed in a bath containing about 400 parts concentrated acetic anhydride, and the mixture agitated, preferably at not to exceed 35° C., action being continued until an apparently homogeneous mixture results, and substantially no unacted upon fibers are visible under low power magnification. If the acetylating mixture is too viscous it may be thinned with a cellulose acetate solvent as acetic acid.

During acetation, oxygen in the form of a plurality of small streams of air may be contacted with ester esterifiant, as by bubbling air or other source containing oxygen passed in contact with or through the acetylating mixture.

The glutinous mixture may then be stored to "homogenize" or "ripen" for a period, or may be immediately precipitated by contact with cold water if the triacetate form is desired; or it may be acetylated to the acetone-soluble or other solvent stage and then precipitated with water, or the acetylated cellulose may be treated with an amount of water insufficient for precipitation in order to obtain desired solubility constants in the finished cellulose acetate. In any case the acetylated cellulose is freed from reactants by precipitation or by solvent recovery, usually by both in manufacturing operations, and dried at a moderate temperature.

*Example II.—Acetation of starch.* One hundred parts of purified starch of commerce is deprived of substantially all moisture, and wetted with a mixture containing 2 to 3% by weight of 50% to 70% perchloric acid in a mixture of 150 parts anhydrous methanol and 50 parts absolute ethanol, and the mixture stirred repeatedly up to a maximum period of about 4 hours, temperature not being allowed to rise above about 30° and preferably not above 25° C.

The mass is then reduced in weight by pressure to about 125 parts, broken up into a fine powder, and immersed in a mixture of about 300 parts concentrated acetic anhydride and about 300-400 parts anhydrous methyl acetate, or methyl acetate containing about one-third ethyl acetate, agitation being continued during addition of acetating

mixture, and continued at temperature preferably not to exceed 25° C. until a sample withdrawn shows a solubility in alcohol-free chloroform, or other solubility characteristics depending upon the degree of acetylation desired.

The granular mass, still substantially conserving the morphological structure of the original starch, is then washed in water to neutral reaction, centrifugalized and dried at a comparatively low temperature.

*Example III.—Acetation of cellulose in textile form.* One hundred parts by weight of a thin muslin of width and length desired is deprived of moisture until it is substantially anhydrous, and then uniformly impregnated in the cooled condition with a mixture of 100-200 parts anhydrous methanol containing dissolved therein 2% to 3% by weight of iodic acid in concentrated solution for a period of about 5 hours, the cloth being turned or otherwise agitated during the contacting period of catalyst with cellulose.

The preferable amount of methanol to use, and the treatment period of cloth with dissolved iodic acid will depend in a measure upon the weight and other physical characteristics, and the nature of the cloth being treated.

At the expiration of the impregnation or dissemination period, the cloth is placed under pressure or liquid evaporated therefrom until the weight of the cloth has been reduced to under 130% of its original weight, when it is then placed under tension and immersed in a closed container containing 300-350 parts concentrated acetic anhydride and 50-200 parts methyl acetate, the temperature range being kept below about 25° C. Or the cloth may be placed under tension during the period of contact of catalyst with cellulose.

When a sample of cloth removed and purified shows the physical characteristics of "cellulose triacetate" (maximum acetated normal cellulose or thereabouts), the cloth, still under tension, is treated to remove reactants in any suitable manner, and moisture removed therefrom, after which the tension is removed.

In addition to the application of tension during cellulose treatment, physical characteristics as luster may also be modified by passing the acetated cloth into or through a chamber containing volatile solvents, plasticizers or other modifying liquids or solids in vapor form, whereby a degree of incipient gelatinization of the acetated fibers is allowed to take place, in degree depending upon the effect desired, and being modified by the tautness of the fibers during said treatment.

In a modification of the process, also given for illustrative purposes only and with the understanding that the reactants and conditions may be considerably modified, still conserving the essence of this invention, a cotton fabric is taken, or a cotton fabric containing a proportion of linen therein or a proportion of mercerized fabric therein, and which has been degummed by a usual kier boil and bleached to produce standard or normal cellulose of high purity, has its free and combined moisture evaporated therefrom by passage through a suitably ventilated section of a tenter dryer having a temperature sufficiently elevated to extract substantially all the moisture therefrom, but insufficiently high to cause appreciable oxidation or decomposition of the cellulose.

When the moisture content of the fabric has been reduced below 1%, the dehydrated fabric, preferably after being allowed to cool, is passed through a bath comprising sufficient anhydrous methanol containing a mixture of bromic and

iodic acid catalyst to thoroughly impregnate the fabric. After a period of contact between catalyst and fabric, liquid is removed by passage of the fabric between squeeze rolls, and the methanol content of the fabric then further reduced substantially below its saturation point by passing the fabric through a further drier section, so adjusted as to temperature and length that a single passage of fabric therethrough reduces the methanol content in the fabric to between 10% and 30% and preferably 20% to 25% increase on the weight of the goods, and the acid content is approximately 1½% of the weight of the goods. While this impregnation to a satisfactory degree of cellulose with catalyst is normally but a matter of a few minutes, yet more uniform results appear to be obtained where cellulose and catalyst are allowed to contact several hours before esterification is initiated.

The evaporated methanol may be recovered from the drier and condensed.

The fabric is cooled by evaporation of methanol therefrom and is then fed through a solution containing 100 parts concentrated acetic anhydride to 50 parts methyl acetate. It is then passed under tension over rollers in contact with a stream of air.

The acetylation is completed in air and the catalyst or its decomposition products removed from the aceted fiber as by evaporation usually in less than a half hour. The temperature of the bath does not require external thermal control as the rise in temperature is insufficient to degenerate the cellulose, and when the bath contains diluent equal to more than the weight of anhydride, the temperature rise of the bath is negligible.

The fabric is then fed into a washer and washed in water at a temperature not exceeding the esterification temperature. Ordinarily any residual reagents may be completely washed out within 10 minutes with water at a temperature of 15° to 25° C. The product is then in suitable condition for finishing as a textile fabric.

If it is desired to further waterproof the fabric, it may be passed through a confined atmosphere containing a solvent for the cellulose acetate, or the solvent may be uniformly sprayed thereon, then passed through a heating chamber for solvent removal. This induces an incipient gelatinization of the exterior layers of acetated cellulose fabric, and more or less binds the fibers together by the agglutinating action of the dissolved or softened acetate portion.

This invention permits the formation of yarns or textiles of various and contrasting colors or shades of dyeing or printing the cellulose fibers, yarns or fabrics with ordinary cotton dyes which are unaffected by the steps in this invention (such as those which are set or developed, as by acids), prior to esterification thereof, thereby eliminating or minimizing the need of special and expensive dyes ordinarily required for dyeing carbohydrate esters, especially organic esters of cellulose. An application Serial No. 351,913 relating to the art of esterification is co-pending.

What is claimed is:

1. In the art of carbohydrate esterification, the steps which include forming bromine pentoxide in situ in said carbohydrate, acetylating said carbohydrate with bromine pentoxide therein, and stabilizing the bromine pentoxide by oxygen during progress of acetylation.

2. Process for esterifying dried fibrous cellulose comprising impregnating said cellulose with an

oxyacid of a halogen of greater atomic weight than fluorine, said oxyacid containing at least three oxygen atoms dissolved in an aliphatic alcohol containing less than five carbon atoms, afterwards removing a portion of catalyst and alcohol, then esterifying with an esterifying aliphatic anhydride to be combined with the carbohydrate for ester formation, continuing said esterification until the degree of ester formation desired has been attained, then removing reactants therefrom and drying the cellulose ester.

3. Method of acetylating comprising impregnating substantially anhydrous cellulose with substantially anhydrous methanol containing bromic acid, allowing cellulose and bromic acid to contact for a period of time, removing a portion of the liquid by pressure, treating the impregnated cellulose with concentrated acetic anhydride to form bromine pentoxyde by reaction with said anhydride, to form water by reaction with the methanol, and to form an acetic ester by reaction with the cellulose, stabilizing the bromine pentoxyde by contact with oxygen during acetylation, permitting said pentoxyde to volatilize from the esters, then removing reactants and aliphatic ester, finally washing to neutrality and drying.

4. In the art of carbohydrate esterification, the steps which include impregnating carbohydrate with bromic acid in a neutral aliphatic alcohol, then dehydrating bromic acid to its corresponding anhydride, and acetylating carbohydrate with acetic anhydride.

5. Process for esterifying cellulose in fibrous condition and textile form in which all esterifiable components entering therein are substantially anhydrous and the acetated cellulose has fibrous appearance, toughness, flexibility and elasticity of the original cellulose used, comprising impregnating cellulose textile with an oxyacid of a halogen of greater atomic weight than fluorine dispersed in an aliphatic alcohol of relatively low molecular weight but susceptible to esterification to an ester which is a non-solvent of the fibrous cellulose acetate formed, removing a portion of alcohol and acid, then immersing said impregnated cellulose into acetic anhydride containing an aliphatic acetate of the aliphatic alcohol previously used, introducing air into acetating bath, continuing action of acetic anhydride on cellulose until the degree of ester formation desired has been attained, removing reactants, washing to neutrality and finally removing moisture therefrom.

6. Method of acetylating comprising drying cellulose until water content thereof is less than 1%, impregnating said cellulose with methanol having bromic acid dissolved therein, reducing by evaporation the proportion of methanol content of the cellulose below its saturation point, then treating the moistened cellulose with an acetylating reagent.

10 7. In a process for acetating carbohydrate wherein all components entering therein are substantially anhydrous, the step comprising impregnating carbohydrate with an oxyacid of a halogen of greater atomic weight than fluorine dispersed in a monohydric aliphatic alcohol of less than five carbon atoms.

15 8. In a process for acetating cellulose wherein the components entering therein are substantially anhydrous, the step comprising activating said cellulose with bromic acid dissolved in methanol.

ANNETTE HARRIS PRATT.

20 *Administratrix of the Estate of William Beach Pratt, Deceased.*

#### REFERENCES CITED

25 The following references are of record in the file of this patent:

#### UNITED STATES PATENTS

|    | Number    | Name                   | Date           |
|----|-----------|------------------------|----------------|
| 30 | 2,103,018 | Ruperti -----          | Dec. 22, 1937  |
|    | 2,221,184 | Ellis -----            | Nov. 12, 1940  |
|    | 2,170,024 | Heckert -----          | Aug. 22, 1939  |
|    | 2,130,150 | Nathanson -----        | Sept. 13, 1938 |
|    | 2,000,602 | Malm et al. -----      | May 7, 1935    |
|    | 2,076,555 | Fothergill -----       | Apr. 13, 1937  |
| 35 | 1,739,863 | Rosenthal et al. ----- | Dec. 17, 1929  |
|    | 1,746,663 | Leuchs -----           | Feb. 11, 1930  |
|    | 2,045,161 | Mueller et al. -----   | June 23, 1934  |
|    | 2,064,384 | Richter et al. -----   | Dec. 15, 1936  |
|    | 1,236,578 | Lindsay -----          | Aug. 14, 1917  |
| 40 | 1,823,350 | Clarke -----           | Sept. 15, 1931 |
|    | 920,828   | Cross -----            | May 4, 1909    |
|    | 2,010,607 | Ruperti -----          | Aug. 6, 1935   |
|    | 1,678,626 | Jaeger -----           | July 24, 1928  |
| 45 | 2,103,012 | Muller et al. -----    | Dec. 21, 1937  |
|    | 2,175,842 | Koetschel -----        | Oct. 10, 1939  |

#### FOREIGN PATENTS

|    | Number  | Country             | Date          |
|----|---------|---------------------|---------------|
| 50 | 405,825 | Great Britain ----- | Feb. 15, 1934 |
|    | 325,231 | Great Britain ----- | Feb. 13, 1930 |
|    | 525,265 | Great Britain ----- | Aug. 26, 1940 |